

## UNITED STATES PATENT OFFICE

2,413,929

## HEAT-TREATING BATH FOR ALUMINUM

James F. Simpson, Old Greenwich, Conn., assignor to American Cyanamid Company, New York, N. Y., a corporation of Maine

No Drawing. Application May 21, 1945,  
Serial No. 595,069

7 Claims. (Cl. 148—21.1)

1

The present invention relates to the heat treatment of aluminum base alloys and to a salt bath which is adapted, upon fusion, therefor.

Heretofore, aluminum base alloys have been heat treated to improve their mechanical properties in a circulating gas furnace and/or in baths of fused nitrates, particularly sodium nitrate.

Heat treatment of aluminum base alloys by means of circulating gas furnaces has included many disadvantages. The heating has not been rapid, uniform, nor evenly maintained. It has been necessary to heat non-productive articles which carry the aluminum pieces such as trucks, carriages, baskets, hangers, and the like. This type of heat treatment is uneconomical and inefficient.

The use of fused nitrate baths involves the maintenance of a hazard, unwarranted in view of the present invention. Although fused sodium nitrate gives physical properties slightly above the minimum requirements set forth in metallurgical specifications, a bath is maintained which can readily cause violent and/or explosive oxidation of any organic materials which may make contact with it.

The principal object of the present invention is to provide a method and means of heat treating aluminum base alloys which will produce mechanical and physical properties in the alloys treated as good or better than those now obtained by treatment in the usual circulating air furnace or fused nitrate bath, which will have no explosion hazard, which will be chemically inert to the alloy, which will be cheap, and otherwise desirable.

To this end the invention contemplates the heat treating of aluminum base alloys in a molten bath comprising KCNO in predominant quantity. By this expression is meant KCNO alone or in admixture with minor quantities of such salts as KCl, NaCl, KCN, NaCN, NaCNO, MgCl<sub>2</sub>, K<sub>2</sub>CO<sub>3</sub>, or the like. The exact composition of the bath, whether of KCNO alone or in admixture with one or more of the above salts, will in some measure depend upon the temperature required for the

2

desired heat treatment as obviously no treatment in such baths may be had prior to their melting point, which varies considerably. For instance, baths in which aluminum base alloys may be satisfactorily heat treated are given below together with their melting points:

|      | Bath composition                                            | Melting point |
|------|-------------------------------------------------------------|---------------|
| 10   |                                                             | ° F.          |
| 1... | KCNO 100%                                                   | 585-590       |
| 2... | KCl 13%                                                     | 545-550       |
| 3... | KCNO 87%<br>NaCN 13%                                        | 525           |
| 4... | KCNO 86%                                                    | 540           |
| 5... | KCN 14%                                                     | 550           |
| 6... | KCNO 90%                                                    | 550           |
| 15   | NaCl 10%                                                    | 580           |
| 7... | KCNO 88%                                                    | 580           |
| 8... | NaCNO 12%                                                   | 580           |
| 20   | KCNO 88%                                                    | 580           |
| 7... | NaCN 4%<br>NaCNO 8%                                         | 580           |
| 8... | KCNO 73%                                                    | 580           |
| 25   | MgCl <sub>2</sub> 15%<br>K <sub>2</sub> CO <sub>3</sub> 12% | 580           |

While the above composition represents substantially eutectic mixtures, the proportions may be reasonably varied when slightly higher temperatures are desired. Such baths may be used at temperatures varying from their melting point up to a temperature just short of substantial decomposition. While the temperature and time of treatment will vary slightly dependent upon the actual composition and mass of the aluminum base alloy, this is a minor variation, as in all cases it has been found that the temperature and time of treatment is substantially that now used for the same alloys in nitrate baths, and somewhat shorter than in circulating air furnaces.

30 The baths of the present invention for the solution heat treatment of aluminum base alloys are operative between substantially 600° F. and 1050° F. However, the usual procedure is to treat the piece for varying lengths of time at about 900° to 1010° F. and quench it in water for 10 to 30

minutes. The lowest operative temperature is limited by the melting point of the heat-treating bath, and the highest operative temperature is that just below the melting point of the alloy.

Various aluminum alloy compositions and the most advantageous and recommended solution heat-treating time and temperature ranges are given in Table I. It is to be understood that only the principal alloying components other than aluminum are stated in the table. The specific amount of aluminum is omitted, but can easily be figured because impurities exist only in traces, it being understood that the alloy has an aluminum base. The common chemical symbols are used in reference to the alloy components.

TABLE I  
*Aluminum alloys*

| Type    | Composition                          | Temp. range, °F. | Heat treating time |
|---------|--------------------------------------|------------------|--------------------|
| Casting | 4% Cu; 1.5% Mg; 2% Ni                | 940-960          | 5-16 hrs.          |
|         | 4.5% Cu                              | 940-970          | 16-24 hrs.         |
|         | 7% Si; 0.3% Mg                       | 990-1010         | 12-16 hrs.         |
| Wrought | 4% Cu; 0.5% Mg; 0.5% Mg              | 925-950          | 10-90 min.         |
|         | 4.5% Cu; 0.6% Mg; 1.5% Mg            | 910-930          | 15-90 min.         |
|         | 0.7% Si; 1.3% Mg; 0.25% Cr           | 960-980          | 15-45 min.         |
|         | 0.25% Cu; 0.6% Si; 1.0% Mg; 0.25% Cr | 960-980          | 15-45 min.         |
|         |                                      |                  |                    |

Table II shows the amount of corrosion resulting from the solution heat treatment of aluminum alloy sheets whose principal alloying constituents are 4.5% copper, 0.6% manganese, and 1.5% magnesium. The salt bath which is used is composed of 87% KCNO and 13% KCl and is heated to substantially 930° F. while the test pieces are immersed therein for varying periods of time. The pieces are then quenched in tap water for 5 to 10 minutes.

TABLE II  
*Corrosion of aluminum alloy sheet*

| Number of samples | Hours of heat treatment | Average loss in weight |                           | Average penetration, inch/year |
|-------------------|-------------------------|------------------------|---------------------------|--------------------------------|
|                   |                         | Mg./cm. <sup>2</sup>   | Mg./cm. <sup>2</sup> /hr. |                                |
| 4                 | 1/2                     | 0.0116                 | 0.14                      | 0.08                           |
| 2                 | 1/6                     | .018                   | .11                       | .03                            |
| 2                 | 1/6                     | .0185                  | .06                       | .0035                          |
| 2                 | 2/6                     | .0265                  | .04                       | .0005                          |
| 2                 | 1 1/2                   | .062                   | .046                      | -----                          |
| 2                 | 2 1/2                   | .115                   | .043                      | -----                          |
| 1                 | 4 1/2                   | .21                    | .047                      | -----                          |
| 2                 | 20                      | .45                    | .022                      | .0001-0.0002                   |

The salt bath described above is typical of those described earlier in this specification. The corrosion of the aluminum alloy is small and any salts which do adhere to its surface are easily washed off with water.

Table III shows the physical properties of specimens of an aluminum alloy of substantially the same composition when they are individually heat treated in the indicated baths for substantially 30 minutes at substantially 930° F., and quenched in water for 10 to 20 minutes. The tensile strength in pounds per square inch and the per cent elongation in 2 inches on a standard tensile test specimen are given for the strains exerted on both the transversal and longitudinal specimens.

4  
TABLE III  
*Physical and mechanical properties of heat-treated aluminum alloy*

| Run No. | Remarks                                           | Transversal                      |                             | Longitudinal                     |                             |
|---------|---------------------------------------------------|----------------------------------|-----------------------------|----------------------------------|-----------------------------|
|         |                                                   | Tensile strength, 1,000 p. s. i. | Percent elongation in 2 in. | Tensile strength, 1,000 p. s. i. | Percent elongation in 2 in. |
| 10      | Specifications                                    | 62.0                             | 15.0                        | 64.0                             | 13.0                        |
| 15      | 1. NaNO <sub>3</sub> bath                         | 65.0                             | 18.0                        | 66.6                             | 18.6                        |
|         | 2. KCNO bath in an aluminum surfaced pot.         | 64.5                             | 19.2                        | 66.5                             | 18.6                        |
|         | 3. 87KCNO-13KCl bath in an aluminum surfaced pot. | 67.0                             | 21.2                        | 69.5                             | 19.7                        |
| 20      | 4. 87KCNO-13KCl bath in steel pot.                | 65.0                             | 20.5                        | 67.0                             | 20.5                        |
|         | 5. Second run of No. 4 in a clean steel pot.      | 66.0                             | 18.5                        | 68.0                             | 20.0                        |
|         | 6. 87KCNO-13KCl bath in steel pot.                | 67.0                             | 19.0                        | 69.0                             | 18.0                        |
| 25      | Average of No. 3-No. 6 incl.                      | 65.3                             | 19.8                        | 68.4                             | 19.6                        |

It is seen that the non-hazardous KCNO bath is as good as a fused nitrate bath. The values obtained by using an eutectic mixture, KCNO-KCl in this instance, are better than obtained by using a fused NaNO<sub>3</sub> bath.

The duration of the aqueous quench of 10 to 30 minutes is seen to have no appreciable effect upon the properties of the aluminum alloy. Table IV shows the properties obtained from a bath of predominately KCNO and those from a NaNO<sub>3</sub> bath are included for a comparison. The baths are maintained at 920° to 930° F.

TABLE IV  
*Physical properties of aluminum alloys held in quench water for various times after bath treatment*

| Run No. | Heat-treating bath   | Minutes in quenching water | Mechanical properties            |                                |                             |
|---------|----------------------|----------------------------|----------------------------------|--------------------------------|-----------------------------|
|         |                      |                            | Tensile strength, 1,000 p. s. i. | Yield strength, 1,000 p. s. i. | Percent elongation in 2 in. |
| 50      | Specifications       |                            | 62.0                             | 40.0                           | 15.0                        |
| 55      | 1. 87KCNO-13KCl      | 10                         | 65.5                             | 41.0                           | 22.0                        |
|         | 2. do                | 10                         | 67.9                             | 41.4                           | 21.5                        |
|         | 3. do                | 20                         | 65.5                             | 41.4                           | 20.5                        |
|         | 4. do                | 20                         | 65.5                             | 40.7                           | 23.0                        |
|         | 5. do                | 30                         | 68.0                             | 41.4                           | 20.5                        |
|         | 6. do                | 30                         | 68.2                             | 41.4                           | 21.5                        |
| 60      | Average              |                            | 68.2                             | 41.2                           | 21.5                        |
|         | 7. NaNO <sub>3</sub> | 10-20                      | 65.5                             | 41.3                           | 21.0                        |
|         | 8. do                | 10-20                      | 68.1                             | 40.6                           | 20.0                        |
|         | Average              |                            | 66.8                             | 41.0                           | 20.5                        |

Again, from the figures given in Table IV it is seen that the aluminum alloy treated according to the present invention, in a bath predominately KCNO, is superior to that treated by the undesirable fused NaNO<sub>3</sub> bath.

It is surprising that such good properties can be obtained from a heat-treating bath containing a chloride. Some of the bath material clings to the piece when it is removed and quickly transferred to the quench water where this salt dissolves and ionizes to form a solution usually considered corrosive. However, heat-treated pieces

of aluminum alloy show no appreciable drop in their good physical characteristics when allowed to stand for extended periods in simulated quench water having a total salt content as high as 10%. Examination for corrosion showed it to be slight, a fact evident from the maintenance of the excellent physical properties of the aluminum alloy piece.

It should be remembered that in industrial usage it is only necessary to water quench an aluminum alloy piece until its temperature is below 212° F., preferably below 80°-90° F., and the adhering salt is dissolved.

As mentioned earlier in this specification, cast aluminum alloys may be heat treated by salt baths of the present invention. The two alloys which follow are typical of those used in the trade.

Alloy "A" has the following composition, it being understood that aluminum is the base metal:

| Composition    | Percent     |
|----------------|-------------|
| Copper.....    | 4.0 to 5.0. |
| Iron.....      | 1.0 max.    |
| Silicon.....   | 1.2 max.    |
| Zinc.....      | 0.03 max.   |
| Magnesium..... | 0.03 max.   |
| Manganese..... | 0.02 max.   |
| Titanium.....  | 0.02 max.   |
| Others.....    | 0.03 max.   |

Tensile test specimens of alloy "A" are solution heat treated in both nitrate and cyanate-chloride baths for 16 hours at 990 ± 5° F. and quenched in water at 70° F. Table V shows not only the minimum specification but also the physical properties of several specimens. The heat treatment of the aluminum alloy tensile test specimens is performed on pairs cast two at a time in the same flask so that the specimens and results obtained therefrom are comparable.

TABLE V  
Physical properties of aluminum alloy "A"

| Bath                      | Yield strength, p. s. i. | Tensile strength, p. s. i. | Elongation, percent in 2" |
|---------------------------|--------------------------|----------------------------|---------------------------|
| Specification (min.)..... | 21,000                   | 32,000                     | 3.0                       |
| NaNO <sub>3</sub> .....   | 23,200                   | 37,900                     | 5.0                       |
| 87KCNO-13KCl.....         | 23,100                   | 43,000                     | 6.0                       |
| NaNO <sub>3</sub> .....   | 27,750                   | 40,150                     | 4.5                       |
| 87KCNO-13KCl.....         | 27,850                   | 43,350                     | 8.0                       |

It is seen that the yield strength of tensile test specimens heat treated by the nitrate and cyanate-chloride baths are substantially equivalent per paired specimens, but both tensile strength and the per cent elongation in 2" are higher for specimens heat treated by salt baths of this invention.

Alloy "B" has the following composition, it being understood that aluminum is the base metal:

| Composition    | Percent       |
|----------------|---------------|
| Copper.....    | 0.20 max.     |
| Iron.....      | 0.50 max.     |
| Silicon.....   | 6.5 to 7.5.   |
| Magnesium..... | 0.20 to 0.40. |
| Others.....    | 0.03 max.     |

Tensile test specimens of alloy "B" are solution heat treated in both nitrate and cyanate-chloride baths for 12 hours at 990 ± 5° F. and quenched in water at 70° F. Table VI shows not only the minimum specification but also the physical properties of several samples. The heat treatment of the aluminum tensile test specimen is performed on pairs cast two at a time in the same flask so that the specimens and results obtained therefrom will be comparable.

TABLE VI  
Physical properties of aluminum alloy "B"

| Bath                      | Yield strength, p. s. i. | Tensile strength, p. s. i. | Elongation, percent in 2" |
|---------------------------|--------------------------|----------------------------|---------------------------|
| Specification (min.)..... | 20,000                   | 30,000                     | 3.0                       |
| NaNO <sub>3</sub> .....   | 31,000                   | 36,100                     | 2.5                       |
| 87KCNO-13KCl.....         | 33,750                   | 36,100                     | 2.5                       |
| NaNO <sub>3</sub> .....   | 26,000                   | 39,750                     | 4.0                       |
| 87KCNO-13KCl.....         | 33,700                   | 40,200                     | 4.0                       |

It is seen that for this alloy both the tensile strength and per cent elongation in 2" are substantially equal per paired tensile test specimen but that the yield strengths are greater for specimens treated in the cyanate baths of the present invention.

In both cast alloys, "A" and "B," the properties are as good or better than those obtained by heat treatment with the hazardous nitrate bath.

While the invention has been described with particular reference to specific embodiments, it is to be understood that it is not to be limited thereto but is to be construed broadly and restricted solely by the scope of the appended claims.

I claim:

1. A method of heat treating an aluminum base alloy work piece which includes the steps of immersing the same in a molten bath predominately of KCNO at a solution heat-treating temperature until the distribution of the alloy components has been improved, removing the work piece from the bath, and water quenching the same.

2. A method of heat treating an aluminum base alloy work piece which includes the steps of immersing the same in a molten bath predominately of KCNO and also containing KCl at a solution heat-treating temperature until the distribution of the alloy components has been improved, removing the work piece from the bath, and water quenching the same.

3. The method of claim 2 in which the bath contains substantially 87% KCNO and substantially 13% KCl.

4. The method of claim 2 in which the bath temperature is from 900° to 1010° F.

5. The method of claim 2 in which a wrought aluminum base alloy is solution heat treated at from 900° to 1010° F. for 10 to 90 minutes.

6. The method of claim 2 in which a cast aluminum base alloy is solution heat treated at from 900° to 1010° F. for 5 to 24 hours.

7. A molten bath including substantially 87% KCNO and substantially 13% KCl.